

## UNITED STATES PATENT OFFICE

1,932,032

## CONTINUOUS CARBURIZING PROCESS

Roysel J. Cowan, Toledo, Ohio, assignor to Surface Combustion Corporation, Toledo, Ohio, a corporation of New York

No Drawing. Application January 28, 1932  
Serial No. 589,539

7 Claims. (Cl. 148—17)

This invention relates to a method of carburizing metal, the present application being a continuation in part of my application Ser. No. 537,873, filed May 16, 1931.

5 The present invention has for its object to provide a commercially practical continuous carburizing process wherein a hydrocarbon gas or vapor may be successfully used and withal to provide a process which among other advantages shall 10 give (1) control of the carbon content of the case produced, (2) uniformity of results, (3) rapidity of carburization, (4) excellence of diffusion between case and core, (5) simplicity of control of the process as a whole, and (6) cleanliness of 15 operation.

In prior carburizing processes making use of a hydrocarbon gas, the precipitation of carbon on the work has been considered objectional and many schemes have been proposed for overcom- 20 ing the objection. In my process, however, the precipitation of carbon on the work during a certain stage of the operation is one of the essential steps of the process. However, notwithstanding the fact that I so conduct the operation 25 as to secure deposition of carbon on the work, the work before emerging from the heat-treating or carburizing chamber is in a clean condition and in fact is almost as bright and clean as before it was carburized. This cleanliness of the 30 work following carburizing is something new and quite revolutionary in the art of carburizing and quite apart from other advantages of the process has distinctive merit.

Among the various steps of my process, one 35 of the important steps is that of passing the work to be carburized and the carburizing gas in the same direction through successive heat zones maintained at different temperatures, the first zone being the low temperature zone for 40 reasons presently appearing.

The carburizing medium which I employ is a gaseous mixture of a hydrocarbon and a diluent containing an oxidizing agent which latter is preferably carbon dioxide although not necessarily exclusively so.

50 The temperature of the low temperature zone is such as will cause decomposition of the hydrocarbon with the liberation of soot (amorphous carbon) in the presence of a catalyst, such temperature being less than carburizing temperature and ranging between 1200 and 1500 deg. F. The catalyst in the present invention is the metal to be carburized. During the passage of the work or metal through said low temperature zone, it receives a deposit of soot (amorphous carbon) re-

sulting from the cracking or decomposition of the major portion of the hydrocarbon passing through said zone.

The temperature of the high temperature zone is the usual carburizing temperature which ranges 60 between 1550 and 1800 deg. F. Following the deposition of carbon on the work in the low temperature zone, the work with its deposit of carbon passes into the high temperature zone. In the high temperature zone, the deposited carbon on the work is completely oxidized with the formation of carbon monoxide with resultant carburization of the metal. The next step is that of carbide diffusion and such diffusion is accomplished by retaining the work in said high temperature zone for the required period, it being 65 understood that the high temperature zone is of such length that following oxidation of the carbon on the work, the work must still move a substantial distance before reaching the outlet 70 end of said zone. As soon as the work emerges 75 from the high temperature zone, it may be directly quenched or otherwise heat-treated, the cleanliness of the work facilitating further heat-treatment.

In order that the process may be efficiently conducted, it is essential that the precipitation of carbon in the low temperature zone occur on the work itself and not on the walls of the muffle. To this end, the said low temperature zone or 80 portion of the muffle is made of a non-catalytic material. So called "calorized" alloy, that is, iron or steel with a surface of aluminum oxide 85 is such a non-catalytic material and may be used. A chrome-iron alloy devoid of nickel also 90 serves the purpose.

While the high temperature portion of the muffle may be made of the same material as the low temperature portion thereof, namely, a non-catalytic material, nevertheless it is preferred to 95 make said high temperature portion of a material which is more resistant to carburization, a suitable material for that purpose being chrome-nickel-iron alloy.

From what has been stated, it will be readily 100 appreciated that from the standpoint of chemical reaction the high temperature zone may be considered as comprising two main reaction zones, namely, a carburizing zone and a diffusion zone. The order of the zones of the heating chamber as a whole, in the order of their occurrence, are (1) a zone of carbon precipitation, (2) a carburizing zone and (3) a diffusion zone where the carbides in the surface layer of the work diffuse 105 inwardly towards the core of the work.

The relative proportions of hydrocarbon and diluent in the carburizing medium will be so controlled as to (1) insure the desired amount of carbon deposition on the work while it is within 5 the low temperature zone; (2) insure the proper amount of oxidizing agent necessary to oxidize said carbon in the high temperature zone, and (3) insure an atmosphere that will not have any 10 decarburizing effect on the work following oxidation of said carbon and while carbide diffusion is taking place.

The hydrocarbon constituent of said carburizing medium may be any of the well known hydrocarbon gases such as manufactured city gas, natural 15 gas, methane, ethane, propane, butane, acetylene or other saturated or unsaturated hydrocarbons having the property of decomposing with the liberation of soot when heated under proper 20 conditions in the presence of a catalyst such as iron or steel. While I prefer to use hydrocarbon gas as such, nevertheless it is within the scope of the invention to vaporize liquid hydrocarbons and utilize the vapors in the same way that the hydrocarbon gas is used.

25 The diluent for the hydrocarbon is preferably dehydrated or partially dehydrated gaseous products of combustion (hereinafter also termed "flue gas") whereof carbon dioxide constitutes say from 8 to 15%. The carbon dioxide constitutes 30 the oxidizing agent for oxidizing the carbon on the work in the high temperature zone. While relatively minute quantities of water vapor and oxygen in the diluent are not harmful and may in fact be desirable, nevertheless it is preferred 35 from the standpoint of better control of the oxidizing agent to dehydrate the flue gas. From the standpoint of uniformity of composition of the flue gas, it is preferred to generate it by burning a mixture of air and gas in proportions for complete 40 combustion of the gas.

The amount of carbon deposition on the work in the low temperature zone can be increased or decreased by increasing or decreasing, respectively, the ratio between the diluent and the hydrocarbon. In other words, the greater the percentage 45 of hydrocarbon in said medium the greater will be the amount of carbon deposition in a given time. The amount of carbon deposition can also be varied by varying the rate of flow of said carburizing medium through the muffle.

Until the work passes into the high temperature zone the oxidizing agent will have no appreciable oxidizing effect on the deposited carbon. It may, however, have some slight oxidizing effect 55 on the work itself, but such oxidation is considered to be beneficial in the later reactions at higher temperatures.

As previously stated, the carburizing gas is caused to flow through the muffle from the low 60 to the high temperature zone, it being remembered that the work is also caused to move from the low to the high temperature zone.

The time required to completely oxidize said carbon on the work in the high temperature zone will, of course, depend upon the kind and amount 65 of oxidizing agent in said diluent. Since the relative percentages of nitrogen and oxidizing agent in the diluent have no effect on the rate of carbon deposition in the low temperature zone (such rate being controlled by the relative percentages of hydrocarbon and diluent), the rate of oxidation of said carbon on the work in the high temperature zone may be controlled by increasing the percentage of oxidizing agent in the 70 diluent as by increasing its carbon dioxide con-

tent or by adding water vapor or oxygen or both. When said diluent is flue gas the composition of the latter may be readily controlled by varying the degree of dehydration or by burning the fuel from which the flue gas is produced with an excess of air. 80

As already stated the final step in the process after the deposited carbon has been oxidized with resultant carburization of the work is the diffusing of the carbide into the work. This is effected 85 by allowing the work to remain in the high temperature zone for an appropriate period in an atmosphere which is non-decarburizing. In the present invention decarburization is effectively prevented by the presence of hydrocarbon gas in the high temperature zone, it being understood 90 that some of the hydrocarbon introduced into the muffle does not decompose in the time available. As is well known to those skilled in the art, there is a definite amount of hydrocarbon gas required 95 by each carbide concentration in the steel to form a "neutral" so-called atmosphere around the steel to prevent decarburization. Thus at a temperature of 1700° F., a steel containing 18/100% carbon will be at equilibrium in a hydrogen atmosphere with about 25/100% natural gas; if the steel contains 59/100% carbon the equilibrium ratio is 85/100% natural gas while if the steel contains 95/100% carbon the ratio is 1½% natural 100 gas. Ratios higher than these will add carbon to the steel while a lower ratio will remove carbon. The exact ratio is affected by the temperature of the operation and the type of hydrocarbon in the atmosphere and is lowered as the temperature is raised. It is a simple matter in 105 the present invention to maintain the necessary hydrocarbon gas in the high temperature zone to offset any decarburizing effect, it being merely necessary to increase the ratio between the hydrocarbon and the oxidizing agent in the car- 110 burizing medium admitted to the muffle. 115

While it is preferred to utilize flue gas as a combined diluent and oxidizing agent, nevertheless it is within the scope of the invention to prepare the diluent by mixing nitrogen and carbon dioxide or other oxidizing agent from separate sources of supply. 120

An important feature of the present invention is the manner in which any established condition dependent upon the characteristics of the carburizing mixture may be controlled and maintained. The effluent gases from the high temperature zone contain combustible constituents. By burning a constant amount of these gases in the open air in any suitable manner and utilizing 125 a thermocouple to indicate the temperature, a constant temperature will indicate an unvarying condition. Other things being equal, a variation in temperature will indicate a change in the ratio of hydrocarbon to diluent in the mixture. If the 130 temperature falls, it is an indication that more hydrocarbon is required to maintain the required condition in the heat treating chamber and vice versa. By proper instrumentalities operable by the temperature variations, the proportion of 135 hydrocarbon gas and diluent in said mixture may be controlled. 140

While the maintenance of any particular pressure within the muffle is not essential to the successful operation of the process, nevertheless it 145 has been found that the rate of reaction is increased as the pressure is increased, and consequently it is within the scope of the invention to maintain such pressure within the muffle as may be desired. It will, of course, be understood 150

- that in any event some pressure above atmospheric will be maintained to exclude the entry of air into the muffle as through the charging and discharging ends thereof.
- 5 In practical operation the muffle may be provided with a vestibule at each end to prevent the entry of air into the muffle proper during charging and discharging of the muffle. The means for conveying the work through the muffle may take various forms depending upon the character of the work to be carburized. For the purpose of heating the muffle in a manner to maintain said temperature zones, the muffle may be surrounded by a combustion chamber 10 which may be divided by a partition to form two chambers corresponding to the high and low temperature zones, respectively, each combustion chamber being independently fired and controlled.
- 15 As an indication of the relative lengths of the low and high temperature zones of the muffle it may be stated that in one commercial installation the low temperature portion of the muffle is approximately six feet in length and the high temperature zone fourteen feet. In this installation, a case depth of 40/1000 inches was obtained by holding the work at a carburizing temperature of 1650 deg. F. for a period of three hours. Of said case about 10/1000 inches was 20 hypereutectoidal. The steel used for carburizing was S. A. E. 1020, namely .20% carbon steel. To obtain said case it was found necessary to use as the carburizing medium approximately seventy-five cubic feet per hour of natural gas and 25 seventy-five cubic feet per hour of flue gas containing twelve per cent carbon dioxide. With a furnace containing a muffle twenty feet long, exclusive of vestibules at both ends, the muffle being twenty seven inches wide by fourteen 30 inches high, the production of carburized steel was found to be four hundred fifty pounds per hour. This rate of production is more than twice that possible with a furnace of the same length using solid carburizing medium.
- 35 45 What I claim as new is:
1. In the art of carburizing metal with a carburizing gas, the steps comprising passing the gas and the metal in the same direction through successive heat zones in a single chamber, the first of said zones being maintained at a lower temperature than the succeeding zone and being less active as a catalyst than steel in assisting in the thermal decomposition of a hydrocarbon gas with the liberation of soot, the said succeeding zone being maintained at carburizing temperature.
  2. In the art of carburizing metal with a carburizing gas, the steps comprising passing the gas and the metal in the same direction through successive heat zones in a single chamber, the first of said zones being maintained at a lower 40 temperature than the succeeding zone and being less active as a catalyst than steel in assisting in the thermal decomposition of a hydrocarbon gas with the liberation of soot, the said succeeding zone being maintained at carburizing temperature and the said carburizing gas comprising a hydrocarbon, an inert diluent and a gas that will oxidize carbon.
- 45 50 55 60 65 70 75 80 85 90 95 100 105 110 115 120 125 130 135
- temperature than the succeeding zone and being less active as a catalyst than steel in assisting in the thermal decomposition of a hydrocarbon gas with the liberation of soot, the said succeeding zone being maintained at carburizing temperature and the said carburizing gas comprising a hydrocarbon, an inert diluent and a gas that will oxidize carbon.
3. In the art of carburizing metal with a carburizing gas, the steps comprising passing the gas and the metal in the same direction through successive heat zones in a single chamber, the first of said zones being maintained at a lower temperature than the succeeding zone and being less active as a catalyst than steel in assisting in the thermal decomposition of a hydrocarbon gas with the liberation of soot, the said succeeding zone being maintained at carburizing temperature and the said carburizing gas comprising a hydrocarbon and flue gas.
4. In the art of carburizing metal, the steps comprising first coating the metal with soot, then heating the metal to carburizing temperature and while the metal is at carburizing temperature subjecting it to the combined action of a gas comprising a gas that will oxidize the soot and a hydrocarbon gas that has previously been subjected to thermal decomposition with the liberation of carbon.
5. The method of carburizing metal which comprises first coating the metal with soot while it is coming up to carburizing temperature, such coating being formed by thermally decomposing in the presence of the metal a hydrocarbon gas, and thereafter subjecting the metal while at carburizing temperature to the combined action of the gases remaining after the thermal decomposition of the hydrocarbon gas and a gas that will oxidize the soot.
6. The method of carburizing metal which comprises first coating the metal with soot while it is coming up to carburizing temperature, such coating being formed by thermally decomposing in the presence of the metal a hydrocarbon gas diluted with flue gas, and thereafter subjecting the metal while at carburizing temperature to the action of the gases remaining after the thermal decomposition of the hydrocarbon gas.
7. The method of carburizing metal which comprises first coating the metal with soot while it is coming up to carburizing temperature, such coating being formed by thermally decomposing a hydrocarbon gas in the presence of the metal and in an environment that is less active as a catalyst than steel in assisting in such decomposition, and thereafter subjecting the metal while at carburizing temperature to the combined action of the gases remaining after the thermal decomposition of the hydrocarbon gas and a gas that will oxidize the soot.

ROYSEL J. COWAN.